

H. FOERSTERLING & A. L. HALVORSEN.  
PROCESS OF EXTRACTING VALUES FROM ORES.  
APPLICATION FILED JUNE 3, 1914.

1,164,636.

Patented Dec. 21, 1915.

Fig. 2



Fig. 1



WITNESSES

K. M. Le Card  
S. M. Braeden

Heinz Foersterling  
Arthur L. Halvorsen  
INVENTORS  
BY Nestick & Kee  
their ATTORNEYS

# UNITED STATES PATENT OFFICE.

HANS FOERSTERLING AND ARTHUR LUDWICK HALVORSEN, OF PERTH AMBOY, NEW JERSEY, ASSIGNEES TO THE HOESSLER & HASSLACHER CHEMICAL CO., OF NEW YORK, N. Y., A CORPORATION OF NEW YORK.

## PROCESS OF EXTRACTING VALUES FROM ORES.

1,164,636.

Specification of Letters Patent. Patented Dec. 21, 1915.

Application filed June 2, 1913. Serial No. 842,569.

To all whom it may concern:

Be it known that we, HANS FOERSTERLING, a subject of the Emperor of Germany, and ARTHUR LUDWICK HALVORSEN, a subject of the 5 King of Norway, both residents of the city of Perth Amboy, county of Middlesex, and State of New Jersey, have invented certain new and useful Improvements in Processes of Extracting Values from Ores, 10 of which the following is a specification.

This invention relates to improvements in processes for the treatment of ores and more particularly to a process for extracting values from ores containing copper, silver 15 or gold, etc., the object of our invention being to provide a process for producing metals by treating ore so that the entire metal content of same is obtained.

With these and other objects in view the 20 invention consists in certain novel steps in the process of treating the ores with suitable cyanid solutions in the presence or absence of mercury and to precipitate the metal from the aforesaid solutions by means of 25 alkali metals.

It is known that metallic Na may be suitably diluted with Hg so that it will at a 30 convenient rate of reaction replace various metals in their respective combinations, such as released in immediate contact with Hg, entering into the Hg forming the respective amalgams. As a practical demonstration may be taken the following acknowledged equation:



Reactions as represented by the above or 40 analogous equations would seem to be of possible importance in the mining industry for precipitation of metals from solutions, especially from cyanid solutions. The fact that such reactions have not to any extent been utilized in the mills may probably be explained by difficulties in application.

45 Among such difficulties may be mentioned: Various undesirable by-reactions are facilitated by the high reaction pressure of Na; it is necessary, but under certain circumstances difficult or impossible, to keep the 50 Na strength of the alloy or amalgam constant or varying within the desired limits; in case of Hg being used as diluting agent

it is difficult to get a reasonably large continuously active surface capacity per certain weight of Hg in use.

As it is a well known fact that all the hydrometallurgical processes for the extraction of copper ores labor under certain disadvantages and as especially in the extraction of copper all the advantages of our 60 process are easily seen we will particularly refer in the description by way of example to the extraction of copper though gold, silver, etc., show an analogous behavior.

In describing the invention reference is 65 had to the accompanying drawing of which—

Figure 1 is a longitudinal and Fig. 2 is a cross sectional view of one form of the apparatus we prefer to use in the operation of 70 the process.

The apparatus shown in Figs. 1 and 2 consists of a cylindrical casing 1 made preferably of soft steel, an axis 2 being centrally located in suitable journals 3 and 4 75 and protruding on either side from the plates 5 and 6 of the casing. The axis 2 bears a closed drum 7 on which, at a small distance from each other, are provided annular plates 8 of soft steel with perforations 80 8<sup>a</sup> for the passage of the solution. The upper part of the casing is furthermore provided with two pipes 9 and 10 through which, respectively, liquors may enter and leave, whereas pipe 11 at the top of the casing 85 serves as an exit for gases. At the bottom of the casing we have provided a kind of pocket 12, a pipe 13 permitting admission of materials into said pocket 12.

For the better understanding of our invention we will now describe in connection 90 with the apparatus disclosed above some examples of the precipitation of metals from the cyanid solution by means of metallic sodium.

Example 1: Our process is of great importance for the reduction of copper from its ores, inasmuch as cyanid solution is known to be a good solvent of copper in its free metallic state as well as of both natural 100 and artificial copper oxid. For the extraction of copper from ore, same is treated with cyanid solutions so that the dissolution of metallic copper or suitably reduced copper

oxids respectively goes on according to the following equations:

1.  $\text{Cu}_2 + (\text{NaCN})_{x-2} + 2\text{H}_2\text{O} = \text{Cu}_2(\text{CN})_2(\text{NaCN})_{x-2} + 2\text{NaOH} + 2\text{H}_2$
2.  $\text{Cu}_2\text{O} + \text{NaCN}_x + \text{H}_2\text{O} = \text{Cu}_2(\text{CN})_2(\text{NaCN})_{x-2} + 2\text{NaOH}$

In the meantime we charge the apparatus with 1300 lbs. of mercury and a small quantity of sodium metal, the latter producing the well-known amalgam. After feeding in the metallic sodium the soft steel plates 8 on drum 7 are rotated by any suitable power arrangement acting on axis 2. The apparatus thus being started the cyanid solution "saturated" with copper from the ore and hereinafter referred to as the "pregnant" solution is admitted through pipe 9 into the casing of the precipitating apparatus. From Fig. 2 it is easily seen that the plates, mechanically and chemically cleansed, are partly submerged in the mercury 16 and by rotating they soon become covered on their surfaces with a film of adhering amalgam. The steel plates, after emerging from the sodium-mercury amalgam, carry a film of such sodium-mercury amalgam into the pregnant solution thus continuously exposing a minute quantity of metallic sodium to the pregnant solution thereby causing interaction between the contents of the solution and the sodium according to the equation:



The precipitation of the copper is favorably influenced by the vigorous agitation of the cyanid solution by means of the rotation of the enfilmed soft steel plates. The "barren" solution, which has been deprived of part of its copper content, is continuously discharged through pipe 10 and is enriched with copper by extracting same from the ore, and the solution, now being in pregnant state again, is then returned to the precipitating apparatus and so on. alternately. Gases may eventually escape through pipe 11. The solution passes the apparatus at the rate of 100 tons per 24 hours; to show the rapidity of the precipitating process we may state that it would be sufficient to pass a certain particle of the solution within about one minute through the apparatus. Metallic sodium, suitably in the form of its amalgam, is simultaneously fed through pipe 13 at the rate of approximately 350 lbs. per 24 hours. The copper amalgam is discharged through pipe 15 in dilute form at a rate which may be varied. The copper amalgam is separated for instance, by filtering, into a "liquid" as well as into a "solid" part; the liquid part of the copper amalgam

is again enriched with sodium metal and is then returned to the apparatus through pipe 13, whereas the solid amalgam is subjected to distillation furnishing the copper in solid form and to the mercury thus also recovered 70 sodium metal is added, the amalgam being admitted into the apparatus.

In connection with the aforesaid we wish to state that furthermore the success of the process greatly depends on the ratio of Cu 75 to NaCN in the solution and we have found it best to have the cyanid solution "saturated" with copper, i. e. to have the ratio of Cu to NaCN as high as possible, the NaCN including here both free cyanid and that 80 contained in the copper alkali cyanid.

A desirable solution of good saturation and consequently satisfactory results is obtained by cyaniding ores containing the copper values as  $\text{Cu}_2\text{O}$ ; a copper ore having the 85 copper in the form of  $\text{Cu}_2\text{O}$  is treated for instance with a 2.5% NaCN solution and a pregnant solution containing 1.15% Cu is obtained, i. e. the ratio of total Cu to total 90 sodium cyanid is 1 to 2.17. The success of the precipitation is all the greater the higher the ratio of Cu to NaCN. It is therefore best to withdraw the copper cyanid solution from the precipitation apparatus when so 95 much copper has been precipitated out of the solution that the ratio of Cu to NaCN is getting low, for instance about 1 to 3; in this case the "barren" solution is reused for extraction until again saturated and thus continuously passed through the cycle. 100

The circumstances accompanying the treatment of ore containing the copper in the form of  $\text{Cu}_2\text{O}$  suggest to reduce cupric ore to  $\text{Cu}_2\text{O}$ . In case a sulfid ore is to be worked up same may be therefore first submitted to 105 an oxidizing and then to a reducing roast in order to bring the ore into such favorable state for treatment by our process.

By the process as described the copper is recovered by dissolution in cyanid solution 110 followed by the precipitation of the dissolved copper and liberation of the cyanid through reaction with alkali metal suitably alloyed with mercury, the total theoretical consumption of alkali metal being 36 lbs. of 115 Na per 100 lbs. of Cu extracted from the ore, precipitated from the solution and recovered as metallic copper. With a reduced carbonate oxid copper ore or an ore containing native copper in simultaneous contact with cyanid solution and mercury or cyanid solution and alkali amalgam, after the surfaces of the reduced metallic particles have become chemically cleansed by the dissolving 120 action of the cyanid solution, such particles 125 pass directly from the ore into the mercury by direct amalgamation. By utilizing this characteristic property in conjunction with the extraction by cyanid a large part of the ore or copper value is recovered without the 130

above chemical consumption, the chemical consumption per total amount of recovered copper being thereby decreased accordingly.

Example 2: For the reduction of silver and relatively small quantities of gold from its ore we treat the latter in suitable tanks with sodium cyanid solution until we obtain 100 tons of a solution containing silver and gold cyanid in the form of their double salt with sodium cyanid, the solution showing per ton for instance, a content of 8.5 oz. silver, 0.095 oz. gold, 3.7 lbs. free NaCN and 0.5 lb. of  $\text{Ca}(\text{OH})_2$ . We admit the cyanid solution referred to above through pipe 9 into the precipitation apparatus which was used in Example 1 for precipitating copper. Also here a film of sodium amalgam is lifted while adhering to the soft steel plates when emerging from the sodium amalgam, thus causing interaction between the metallic sodium of the amalgam and the silver cyanid contained in the solution whereby metallic silver is precipitated according to the equation:



and is absorbed by the mercury forming silver amalgam.

Like the copper amalgam in Example 1 the silver amalgam is withdrawn from the precipitating vessel through pipe 15 and subsequently separated into "liquid" and "solid" amalgam; the solid amalgam is subjected to distillation to obtain the silver as well as the mercury in its free state. To the mercury thus recovered as well as to the liquid silver amalgam is added a new charge of sodium and the sodium amalgam thus obtained is returned to the precipitation vessel as the situation may require. The sodium is thus fed, preferably in the form of its amalgam at the rate of 90 lbs. per day; the cyanid solution to be treated passing the vessel at the rate of 100 tons per day, while the rate for withdrawing silver amalgam may be regulated according to the arrangement used for sodium feed and varied from about 35-350 lbs. per hour. The barren solution discharged from the precipitating apparatus contains per ton a value of \$0.07 in  $\text{Ag} + \text{Au}$ , 4.1 lbs. of free sodium cyanid and 1.7 lbs. equivalent  $\text{Ca}(\text{OH})_2$ .

The efficiency of our process is evident from the consideration of the values contained in the pregnant solution and those left in the barren solution as discharged from the precipitating apparatus approximately 1-2 minutes after entrance into the same. On the basis of \$60 and \$20 respectively for silver and gold prices the value of the pregnant solution per ton amounts to \$7.00 whereas the barren solution carries only a value of \$.07 per ton, thus showing a precipitation efficiency of 99%.

65 The advantages of our invention are great

and important inasmuch as the process outlined above is very simple in its operation and free from complications; it is especially important for its great efficiency in completely and economically recovering the entire metal content of suitable ores by applying a relatively small quantity of mercury in continuous use. In our case one may recover for instance all the values of gold, silver and copper simultaneously whereas in the former art much cyanid was spent on an ore containing the three metals, in dissolving same all together, whereas, however, copper could not be recovered unless under great difficulties resulting in great loss of materials, labor and time.

In our process no cyanid is lost as it is always recovered as seen from the equation:



The cyanid originally applied is therefore liberated again and replenished to circulate in a cycle between the cyanidation and precipitation apparatus.

Though the soft steel plates offer an enormous surface to the solution notwithstanding, the only source of loss of metallic sodium which may be sustained in our process by interaction with water, is reduced to a minimum owing to the extremely small percentage of metallic sodium in the film of sodium amalgam adhering to the carrying means, such as plates, etc., made of soft steel or other suitable material.

It is of considerable importance for the economic success of our process that we are able to prevent further losses by oxidizing reactions attacking the sodium in the amalgam as well as the cyanid in the solution. An oxidizing action may be due to oxygen *in statu nascendi* and as the formation of such oxygen is invited if  $\text{CuO}$  is dissolved in sodium cyanid, we therefore prefer all the more to reduce the copper compounds for treatment by our process; by furthermore incasing the sodium amalgam entirely in a closed vessel we also exclude the harmful influences of atmospheric oxygen from the sodium amalgam.

A further and rather important advantage of our process consists in the purity of the metals obtained by the precipitation process, for though of course according to the various metallic contents of an ore a mixture of metals is obtained, said mixture is particularly free from sulfur, phosphorus, silicon and other like impurities the removal of which by chemical methods is known to cause great expense in time and money.

It is obvious that our process is not restricted to the reduction of gold, silver and copper to their metallic state as any other metal which itself as well as its oxid dissolves in cyanid solution is equally amenable to our process and we therefore claim such

other metals as coming within the scope of our invention.

Whenever we speak of a "film" we mean also to include a plurality of films or such a large though irregular surface as is formed upon any other suitable carrying means desirable for the purposes of our invention. As such a film or other form offering like advantage may be produced by various means and as this may be used without deviating from the spirit or sacrificing the advantage of our invention we therefore claim also any such deviation as a part of our invention and coming within the scope of same. Finally we wish to state that whenever we speak of an "alkali metal" we mean to include as well an alkali earth metal, mixtures of alkali metals or of alkali and alkali earth metals.

20. We claim:

1. The process of extracting values from ores consisting in treating the ore with a solution of a cyanid capable of forming a soluble cyanid salt with the value and reacting upon the value-charged solution with a moving, adherent film of an amalgam.

2. The process of extracting values from ores consisting in treating the ore with a solution of a cyanid capable of forming a soluble cyanid salt with the value and reacting upon the value-charged solution with a vertical, adherent, rotating film of amalgam.

3. The process of extracting values from ores consisting in treating the ore with a solution of a cyanid capable of forming a soluble cyanid salt with the value and reacting upon the value-charged solution with a moving, adherent film of an amalgam capable of displacing the value in the solution and of regenerating the original cyanid.

4. The process of extracting values from ores consisting in treating the ore with a solution of a cyanid capable of forming a soluble cyanid salt with the value and reacting upon the value-charged solution with a moving, continuously-renewed, adherent film of an amalgam capable of displacing the value in the solution and of regenerating the original cyanid.

5. The process of extracting values from ores consisting in treating the ore with a solution of a cyanid capable of forming a soluble cyanid salt with the value and reacting upon the value-charged solution with a continuous, moving, adherent film of an amalgam capable of displacing the value in the solution and of regenerating the original cyanid.

6. The process of extracting values from ores consisting in treating the ore with a solution of a cyanid capable of forming a soluble cyanid salt with the value and passing the value-charged solution through and against a series of moving, adherent films of amalgam.

7. The process of extracting values from ores consisting in treating the ore with a solution of a cyanid capable of forming a soluble cyanid salt with the value and passing the value-charged solution horizontally through and against a series of perforated, moving, adherent films of amalgam.

8. The process of extracting values from ores consisting in treating the ore with a solution of a cyanid capable of forming a soluble cyanid salt with the value and passing the value-charged solution horizontally over a surface of amalgam while passing a series of adherent films of amalgam through the solution in the path of its flow over the surface of amalgam.

9. The process of extracting values from ores consisting in treating the ore with a solution of a cyanid capable of forming a soluble cyanid salt with the value, passing the value-charged solution horizontally over a surface of amalgam and through a series of perforated, moving, adherent films of amalgam.

10. The process of extracting values from ores consisting in treating the ore with a solution of a cyanid capable of forming a soluble cyanid salt with the value, passing the value-charged solution horizontally over a surface of amalgam through a series of perforated, vertical, adherent, rotating films of amalgam and constantly renewing said films by passing the same, in their rotation, through a body of amalgam.

11. The process of extracting values from ores consisting in treating the ore with a solution of a cyanid capable of forming a soluble cyanid salt with the value and forcing the value-charged solution over and against a plurality of moving, adherent films of amalgam.

12. The process of extracting values from ores consisting in treating the ore with a solution of a cyanid capable of forming a soluble cyanid salt with the value until said solution is substantially saturated and reacting upon said substantially saturated value-charged solution with a plurality of moving, adherent films of amalgam.

13. The process of extracting values from ores consisting in treating the ore with a solution of a cyanid capable of forming a soluble cyanid salt with the value and reacting upon the value-charged solution, under exclusion of air, with a moving, adherent film of amalgam.

14. The process of extracting values from ores consisting in treating the ore with a solution of a cyanid capable of forming a soluble cyanid salt with the value, reacting upon the value-charged solution with a moving, adherent film of an amalgam capable of displacing the value in the solution and of regenerating the original cyanid, retreating fresh ore with the substantially value-free

and regenerated cyanid and repeating the process in a continuous cycle.

15. The process of extracting values from ores consisting in treating the ore with a solution of a cyanid capable of forming a soluble cyanid salt with the value, reacting upon the value-charged solution with a moving, adherent film of an amalgam capable of displacing the value in the solution and of regenerating the original cyanid, removing a portion of the value from the solution and regenerating the solution from which the value has been removed, retreating fresh ore with the value-depleted and regenerated solution and repeating the process in a continuous cycle.

16. The process of extracting values from ores consisting in treating the ore with a solution capable of forming a soluble salt with the value and reacting upon the value-charged solution with a moving, adherent film of amalgam.

17. The process of extracting values from ores consisting in treating the ore with a solution capable of forming a soluble salt with the value and reacting upon the value-charged solution with a moving, adherent film of an amalgam capable of displacing the value in the solution and of regenerating the original solution.

18. The process of extracting values from ores consisting in treating the ore with a solution capable of forming a soluble salt with the value and reacting upon the value-charged solution with a moving, adherent film of an alkali amalgam capable of displacing the value in the solution and of regenerating the original solution.

19. The process of extracting values from ores consisting in treating the ore with a solution capable of forming a soluble salt with the value, and reacting upon the value-charged solution with a continuous, vertical, adherent, rotating film of alkali amalgam constantly emerging from a well of said amalgam, said amalgam being capable of displacing the value in the solution and of regenerating the original solution.

20. The process of extracting values from ores consisting in treating the ore with a solution of a cyanid capable of forming a soluble cyanid salt with the value and reacting upon the value-charged solution with a continuous, vertical, adherent rotating film of amalgam constantly emerging from a well of said amalgam.

21. The process of extracting values from ores consisting in treating the ore with a solution of a cyanid capable of forming a soluble cyanid salt with the value, reacting upon the value-charged solution with a moving, adherent film of alkali amalgam constantly emerging from a well of said amalgam and continuously maintaining a sub-

stantially constant content of alkali metal in the amalgam.

22. The process of extracting values from ores consisting in treating the ore with a solution of a cyanid capable of forming a soluble cyanid salt with the value, passing the value-charged solution into a well containing an alkali amalgam, carrying a continuous, adherent film of alkali amalgam constantly emerging from said well through said solution and precipitating the value and regenerating the solution by the reaction between said value-charged solution and said amalgam.

23. The process of extracting values from ores consisting in treating the ore with a solution of a cyanid capable of forming a soluble cyanid salt with the value, passing the value-charged solution into a well containing an alkali amalgam, carrying a continuous, adherent film of alkali amalgam constantly emerging from said well through said solution, precipitating the value and regenerating the solution by the reaction between said value-charged solution and said amalgam, withdrawing a portion of the amalgam containing said precipitated metal and maintaining a substantially constant content of alkali metal in the alkali metal amalgam.

24. The process of extracting values from ores consisting in treating the ore with a solution of a cyanid capable of forming a soluble cyanid salt with the value, passing the value-charged solution into a well containing an alkali metal amalgam, carrying a continuous, adherent film of alkali metal amalgam constantly emerging from said well through said solution, reacting upon the solution with the alkali metal of the amalgam to precipitate the value, forming an amalgam of the value and the mercury of the alkali-free amalgam, withdrawing a portion of the amalgam containing said precipitated value and replenishing the alkali metal removed by the reaction in the form of alkali metal amalgam.

25. The process of extracting values from ores consisting in treating the ore with a solution of a cyanid capable of forming a soluble cyanid salt with the value, passing the value-charged solution into a well containing an alkali amalgam, carrying a continuous, adherent film of alkali amalgam constantly emerging from said well through said solution, reacting on the solution with the alkali metal to precipitate a part of the value therefrom, forming an amalgam of the value precipitated and the mercury of the alkali-free amalgam, continuously withdrawing the partly exhausted value-charged solution from the well, treating ore with said partly exhausted value-charged solution, continuously returning said re-

value-charged solution to the well, withdrawing a portion of the amalgam containing the precipitated value, removing said value from said amalgam, recharging the recovered mercury with alkali metal and returning said alkali metal amalgam to the well.

26. The process of extracting values from ores consisting in treating the ore with a solution of sodium cyanid, passing the value-charged solution into a well containing sodium amalgam, carrying a continuous, adherent film of sodium amalgam constantly emerging from said well through said solution, reacting on the solution with the sodium to precipitate a part of the value therefrom and regenerate a proportionate amount of sodium cyanid, forming an amalgam of the value precipitated and the mercury of the sodium-depleted amalgam, continuously withdrawing the partly exhausted value-charged and regenerated solution from the well, treating ore with said partly exhausted value-charged and regenerated solution, continuously returning said regenerated solution to the well, withdrawing a portion of the amalgam containing the precipitated value, removing said value from said amalgam, recharging the recovered mercury with sodium and returning said sodium amalgam to the well.

27. The process of extracting copper from ore consisting in treating the ore with a solution of an alkali metal cyanid capable of forming a soluble cyanid salt with the copper until said solution is substantially saturated, reacting upon the solution with an alkali metal amalgam to precipitate a portion of the copper from the solution and regenerate the alkali metal cyanid, treating ore with the depleted copper-charged and regenerated solution until said solution is substantially saturated and repeating the cycle.

45 28. The process of extracting copper from ore consisting in treating the ore with a solution of sodium cyanid until said solution is substantially saturated, reacting upon the solution with sodium amalgam to precipitate a portion of the copper from the solution and regenerate the sodium cyanid, treating ore with the depleted copper-charged and regenerated sodium cyanid solution until said solution is substantially saturated and repeating the cycle.

29. The process of extracting copper from ore consisting in treating the ore with a solution of an alkali metal cyanid capable of forming a soluble cyanid salt with the copper until said solution is substantially saturated, reacting upon the solution under substantially non-oxidizing conditions with an alkali metal amalgam to precipitate a portion of the copper from the solution and regenerate the alkali metal cyanid, treating

ore with the depleted copper-charged and regenerated solution until said solution is substantially saturated and repeating the cycle.

30. The process of extracting copper from ore consisting in treating the ore with a solution of sodium cyanid until said solution is substantially saturated, reacting upon the solution under substantially non-oxidizing conditions with sodium amalgam to precipitate a portion of the copper from the solution and regenerate the sodium cyanid, treating ore with the depleted copper-charged and regenerated sodium cyanid solution until said solution is substantially saturated and repeating the cycle.

31. The process of extracting copper from ore consisting in treating the ore with a solution of an alkali metal cyanid capable of forming a soluble cyanid salt with the copper until said solution is substantially saturated, reacting upon the solution with an alkali metal amalgam to precipitate a portion of the copper from the solution and regenerate the alkali metal cyanid, treating ore with the depleted copper-charged and regenerated solution until said solution is substantially saturated and repeating the cycle, continuously maintaining a substantially constant content of alkali metal in the amalgam.

32. The process of extracting copper from ore consisting in treating the ore with a solution of sodium cyanid until said solution is substantially saturated, reacting upon the solution with sodium amalgam to precipitate a portion of the copper from the solution and regenerate the sodium cyanid, treating ore with the depleted copper-charged and regenerated sodium cyanid solution until said solution is substantially saturated and repeating the cycle, continuously maintaining a substantially constant content of sodium in the amalgam.

33. The process of extracting copper from ore consisting in bringing the ore into such condition that the copper therein is in the form of cuprous oxid, reacting the cuprous oxid with a solution of an alkali metal cyanid capable of forming a soluble salt with the copper until said solution is substantially saturated, reacting upon the substantially saturated solution with an alkali metal amalgam to precipitate a portion of the copper from the solution and to liberate a corresponding amount of alkali metal to form alkali metal cyanid, treating cuprous oxid with the depleted copper-charged and alkali metal regenerated cyanid solution until said solution is substantially saturated and repeating the cycle.

34. The process of extracting values from ores consisting in recovering non-precious metals from ores with simultaneous recovery of precious metals by first treating the

ore to bring the metals into oxydul and metallic condition, dissolving the metals in that condition by alkali cyanid and precipitating the metals with dilute alkali metal while liberating alkali cyanid.

35. The process of extracting values from ores consisting in recovering non-precious metals from ores with simultaneous recovery of precious metals by first treating the ore to bring a substantial part of the metals into metallic condition, recovering the metals in metallic form by direct amalgamation in the presence of cyanid solution, dissolv-

ing the remainder of the metals in alkali cyanid and precipitating said dissolved metals from the alkali cyanid with dilute alkali metal while liberating a corresponding amount of alkali cyanid.

In testimony whereof we have signed this specification in the presence of two subscribing witnesses.

HANS FOERSTERLING.

ARTHUR LUDWICK HALVORSEN.

Witnesses:

RALPH N. SARGENT,

OTTO K. ZWINZENBERGER.